

# UNITED STATES PATENT OFFICE.

WILLIAM STRUTT, OF PITTSBURGH, PENNSYLVANIA, ASSIGNOR TO WESTINGHOUSE ELECTRIC AND MANUFACTURING COMPANY, A CORPORATION OF PENNSYLVANIA.

## ABRASIVE AND PROCESS OF MAKING THE SAME.

1,324,215.

Specification of Letters Patent.

Patented Dec. 9, 1919.

No Drawing.

Application filed March 4, 1915. Serial No. 12,206.

*To all whom it may concern:*

Be it known that I, WILLIAM STRUTT, a citizen of the United States, and a resident of Pittsburgh, in the county of Allegheny and State of Pennsylvania, have invented a new and useful Improvement in Abrasives and Processes of Making the Same, of which the following is a specification.

My invention relates to the manufacture of abrasive bodies, and it has for one of its objects to provide a simple, inexpensive and effective process of treating abrasive materials for the purpose of greatly increasing their effective life and efficiency.

Another object of my invention is to provide a new and superior abrasive article having superior grinding properties and having, in particular, the property of being self-cleaning, that is to say, of repelling from its surface the particles ground off from the materials to which the abrasive may be applied.

Certain very hard abrasive materials, such as carborundum and corundum, are well adapted for use in the grinding and polishing of metals, and for this purpose they are commonly formed into rectangular blocks of sizes convenient for handling. It is found that, when such abrasive blocks are used to grind relatively soft and malleable materials, such as copper, some of the particles ground off by the abrasive block are retained upon its surface, entering between the fine tooth-like cutting projections of the abrasive, and destroying its cutting power to a considerable extent. When such a block is used thereafter, its effect upon the material being ground is to rub off the surface of the material instead of cutting or grinding it.

I have discovered that the foregoing disadvantage may be overcome by impregnating the abrasive bodies with certain oils, which appear to cause the surfaces of the cutting teeth of the abrasive to repel the fine particles of copper or other such material, and which thereby render the cutting surfaces of the abrasive self-cleaning. The abrasives consequently have a much longer effective life and an increased degree of efficiency.

In carrying out one modification of my

process, I make use of carborundum grinding stones of any ordinary sizes, such as 1 by 2 by 8 inches, and I immerse the stones 55 in a relatively light hydrocarbon machine oil for a considerable time, until the blocks have absorbed as much of the oil as possible. I have found that this maximum absorption takes place in somewhat less than 60 one hundred hours, and I therefore prefer to allow the blocks to soak in the machine oil for about one hundred hours, after which I remove them from the oil and ignite the oil which drips from the surfaces of the 65 blocks. The surface oil should be allowed to burn until oil ceases to drip from the blocks, at which time the flame should be extinguished, and the blocks allowed to cool. They are then ready for use. 70

I have found that carborundum blocks absorb at least 8% of their weight of light hydrocarbon machine oil, and I have also found that the burning treatment, described above, greatly improves the cutting properties of the blocks, although the exact reason for this improvement is not clear. 75

Abrasive blocks prepared in accordance with my invention may be used for grinding soft metals, such as copper, at very high 80 speeds, which has heretofore not been possible with the abrasives commonly used, on account of the surface accumulations of ground material mentioned above. This property of my improved abrasive materials 85 renders them particularly well adapted for use in grinding the commutators of dynamo-electric machines, which must be ground while rotating at high peripheral speeds.

The steps of my process and the materials 90 employed may be variously modified without departing from the principles of my invention, and it is therefore to be understood that my invention is not restricted to the precise process steps and substances 95 mentioned above, but is limited only by the scope of the appended claims.

I claim as my invention:

1. A process of treating bodies of abrasive material that comprises impregnating the 100 bodies with an oil and then burning the adhering oil from the surfaces of the blocks.

2. A process of improving the abrasive properties of carborundum blocks that com-

prises immersing the blocks in a mineral oil until the blocks have absorbed a substantial quantity of the oil, removing the blocks from the oil, igniting the oil adhering to the surfaces of the blocks, and extinguishing the flame when oil ceases to drip from the blocks.

In testimony whereof, I have hereunto subscribed my name this 26th day of Feb., 1915.

WM. STRUTT.

Witnesses:

PARKER NEFF,  
B. B. HINES.